



US007765835B2

(12) **United States Patent**  
**Karayianni et al.**

(10) **Patent No.:** **US 7,765,835 B2**  
(45) **Date of Patent:** **Aug. 3, 2010**

(54) **ELASTIC COMPOSITE YARN, METHODS FOR MAKING THE SAME, AND ARTICLES INCORPORATING THE SAME**

(75) Inventors: **Eleni Karayianni**, Geneva (CH); **Philippe Chaudron**, Sant Julien en Genevois (FR); **George W. Coulston**, Pittsburgh, PA (US)

(73) Assignee: **Textronics, Inc.**, Wilmington, DE (US)

(\*) Notice: Subject to any disclaimer, the term of this patent is extended or adjusted under 35 U.S.C. 154(b) by 180 days.

(21) Appl. No.: **11/719,116**

(22) PCT Filed: **Nov. 8, 2005**

(86) PCT No.: **PCT/IB2005/003345**

§ 371 (c)(1),  
(2), (4) Date: **Jul. 16, 2008**

(87) PCT Pub. No.: **WO2006/051384**

PCT Pub. Date: **May 18, 2006**

(65) **Prior Publication Data**

US 2009/0071196 A1 Mar. 19, 2009

**Related U.S. Application Data**

(60) Provisional application No. 60/627,168, filed on Nov. 15, 2004.

(51) **Int. Cl.**  
**D04B 1/18** (2006.01)

(52) **U.S. Cl.** ..... **66/172 E**  
(58) **Field of Classification Search** ..... **66/170,**  
66/172 E, 202; 57/210, 225, 231

See application file for complete search history.

(56)

**References Cited**

U.S. PATENT DOCUMENTS

|             |         |                  |
|-------------|---------|------------------|
| 3,273,978 A | 9/1966  | Victor           |
| 3,288,175 A | 11/1966 | Valko            |
| 3,336,174 A | 8/1967  | Dyer et al.      |
| 3,354,630 A | 11/1967 | Segal            |
| 3,625,809 A | 12/1971 | Caroselli et al. |
| 3,979,648 A | 9/1976  | Toyoshima et al. |
| 4,160,711 A | 7/1979  | Nishizawa et al. |
| 4,226,076 A | 10/1980 | Griset, Jr.      |
| 4,228,641 A | 10/1980 | O'Neil           |
| 4,234,907 A | 11/1980 | Daniel           |
| 4,239,046 A | 12/1980 | Ong              |
| 4,299,884 A | 11/1981 | Payen et al.     |
| 4,433,536 A | 2/1984  | O'Neil           |
| 4,525,992 A | 7/1985  | Payen et al.     |

(Continued)

FOREIGN PATENT DOCUMENTS

DE 10342787 A1 5/2004

(Continued)

*Primary Examiner*—Danny Worrell  
(74) *Attorney, Agent, or Firm*—Connolly Bove Lodge & Hutz LLP

(57) **ABSTRACT**

An elastic composite yarn comprises a composite core and a composite covering. The composite core comprises an elastic core member and an inelastic functional core member. The composite covering comprises at least an elastic covering member and at least one inelastic covering member surrounding the elastic covering member, such that substantially all of an elongating stress imposed on the composite yarn is carried by the elastic core member and the elastic covering member.

**18 Claims, 10 Drawing Sheets**



## U.S. PATENT DOCUMENTS

|                |         |                    |                      |         |                        |          |
|----------------|---------|--------------------|----------------------|---------|------------------------|----------|
| 4,544,603 A    | 10/1985 | Richards           | 7,059,714 B2 *       | 6/2006  | Kaeding et al. ....    | 428/32.1 |
| 4,572,960 A    | 2/1986  | Ebneth et al.      | 7,135,227 B2         | 11/2006 | Karayianni et al.      |          |
| 4,583,547 A    | 4/1986  | Granek et al.      | 7,147,904 B1         | 12/2006 | Crawford               |          |
| 4,651,163 A    | 3/1987  | Sutera et al.      | 7,240,522 B2 *       | 7/2007  | Kondou et al. ....     | 66/195   |
| 4,654,748 A    | 3/1987  | Rees               | 7,413,802 B2 *       | 8/2008  | Karayianni et al. .... | 57/211   |
| 4,777,789 A    | 10/1988 | Kolmes et al.      | 7,504,127 B2         | 3/2009  | Karayianni et al.      |          |
| 4,813,219 A    | 3/1989  | Rees               | 2002/0050446 A1      | 5/2002  | Antoniazzi             |          |
| 4,878,148 A    | 10/1989 | Hee et al.         | 2002/0130624 A1      | 9/2002  | Nakamura               |          |
| 4,885,663 A    | 12/1989 | Parker             | 2003/0224681 A1      | 12/2003 | Koch                   |          |
| 4,907,132 A    | 3/1990  | Parker             | 2004/0023576 A1      | 2/2004  | Rock et al.            |          |
| 4,929,803 A    | 5/1990  | Yoshida et al.     | 2004/0171284 A1      | 9/2004  | Sweetland et al.       |          |
| 5,042,900 A    | 8/1991  | Parker             | 2004/0209059 A1      | 10/2004 | Foss                   |          |
| 5,102,727 A    | 4/1992  | Pittman et al.     | 2004/0216287 A1      | 11/2004 | Bakker et al.          |          |
| 5,103,504 A    | 4/1992  | Dordevic           | 2004/0235381 A1      | 11/2004 | Iwasaki et al.         |          |
| 5,275,861 A    | 1/1994  | Vaughn             | 2004/0237494 A1      | 12/2004 | Karayianni et al.      |          |
| 5,288,544 A    | 2/1994  | Mallen et al.      | 2005/0282009 A1      | 12/2005 | Nusko et al.           |          |
| 5,503,887 A    | 4/1996  | Diaz et al.        |                      |         |                        |          |
| 5,568,964 A    | 10/1996 | Parker et al.      |                      |         |                        |          |
| 5,632,137 A    | 5/1997  | Kolmes et al.      | EP 0111070 A1        | 6/1984  |                        |          |
| 5,771,027 A    | 6/1998  | Marks et al.       | EP 1 319 741 A1      | 6/2003  |                        |          |
| 5,906,004 A    | 5/1999  | Lebby et al.       | FR 2031797           | 11/1970 |                        |          |
| 5,910,361 A    | 6/1999  | Guevel et al.      | FR 2 745 690 A1      | 9/1997  |                        |          |
| 5,927,060 A    | 7/1999  | Watson             | GB 2156592           | 10/1985 |                        |          |
| 5,968,854 A    | 10/1999 | Akopian et al.     | GB 2361431           | 10/2001 |                        |          |
| 6,105,224 A    | 8/2000  | O'Mara, Jr. et al. | WO WO-92/13352 A1    | 8/1992  |                        |          |
| 6,138,336 A    | 10/2000 | Goineau            | WO 9516877 A1        | 6/1995  |                        |          |
| 6,145,551 A    | 11/2000 | Jayaraman et al.   | WO WO-01/02052 A2    | 1/2001  |                        |          |
| 6,341,504 B1   | 1/2002  | Istook             | WO WO-01/37366 A1    | 5/2001  |                        |          |
| 6,356,238 B1   | 3/2002  | Gainor et al.      | WO WO-01/39326 A1    | 5/2001  |                        |          |
| 6,377,216 B1   | 4/2002  | Cheadle et al.     | WO 0212785 A1        | 2/2002  |                        |          |
| 6,381,482 B1   | 4/2002  | Jayaraman et al.   | WO 02068862 A1       | 9/2002  |                        |          |
| 6,399,879 B1   | 6/2002  | Ueda et al.        | WO WO-02/071935 A1   | 9/2002  |                        |          |
| 6,519,979 B2 * | 2/2003  | Freedman .....     | WO WO-03/094717 A1   | 11/2003 |                        |          |
| 6,581,366 B1   | 6/2003  | Andrews            | WO WO-2004/006700 A1 | 1/2004  |                        |          |
| 6,677,917 B2   | 1/2004  | Van Heerden et al. | WO WO-2004/027132    | 4/2004  |                        |          |
| 6,680,707 B2   | 1/2004  | Allen et al.       | WO 2004057079 A1     | 7/2004  |                        |          |
| 6,701,703 B2 * | 3/2004  | Patrick .....      | WO WO-2004/058346 A1 | 7/2004  |                        |          |
| 6,738,265 B1   | 5/2004  | Svarfvar et al.    | WO 2004097089 A1     | 11/2004 |                        |          |
| 6,803,332 B2   | 10/2004 | Andrews            | WO WO-2004100784 A2  | 11/2004 |                        |          |
| 6,856,715 B1   | 2/2005  | Ebbesen et al.     |                      |         |                        |          |
| 6,970,731 B1   | 11/2005 | Jayaraman et al.   |                      |         |                        |          |

## FOREIGN PATENT DOCUMENTS

|    |                   |         |
|----|-------------------|---------|
| EP | 0111070 A1        | 6/1984  |
| EP | 1 319 741 A1      | 6/2003  |
| FR | 2031797           | 11/1970 |
| FR | 2 745 690 A1      | 9/1997  |
| GB | 2156592           | 10/1985 |
| GB | 2361431           | 10/2001 |
| WO | WO-92/13352 A1    | 8/1992  |
| WO | 9516877 A1        | 6/1995  |
| WO | WO-01/02052 A2    | 1/2001  |
| WO | WO-01/37366 A1    | 5/2001  |
| WO | WO-01/39326 A1    | 5/2001  |
| WO | 0212785 A1        | 2/2002  |
| WO | 02068862 A1       | 9/2002  |
| WO | WO-02/071935 A1   | 9/2002  |
| WO | WO-03/094717 A1   | 11/2003 |
| WO | WO-2004/006700 A1 | 1/2004  |
| WO | WO-2004/027132    | 4/2004  |
| WO | 2004057079 A1     | 7/2004  |
| WO | WO-2004/058346 A1 | 7/2004  |
| WO | 2004097089 A1     | 11/2004 |
| WO | WO-2004100784 A2  | 11/2004 |

\* cited by examiner

*Fig. 1A.**Fig. 1B.*

*Fig. 2*

200 $\mu$ m

*Fig. 4.*

200 $\mu$ m

*Fig.3A.*

100 $\mu$ m

*Fig.3B.*

100 $\mu$ m

*Fig. 5A.**Fig. 5B.*

*Fig. 6A.**Fig. 6B.*

*Fig. 7.*





*Fig.12.*







## 1

**ELASTIC COMPOSITE YARN, METHODS  
FOR MAKING THE SAME, AND ARTICLES  
INCORPORATING THE SAME**

FIELD OF THE INVENTION

The present invention relates to elastified yarns containing high modulus or low bending functional fibers, a process for producing the same, and to stretch fabrics, garments, and other articles incorporating such yarns. The invention also relates to novel elastified yarns made via yarn covering processes in which at least one covering member is, itself, an elastified yarn.

BACKGROUND OF THE INVENTION

Fabrics with functional properties have been disclosed for use in textile yarns. Examples include metallic yarns that can be used for carrying electrical current, performing an anti-static electricity function, or providing shielding from electric fields. Such yarns or fibers can, for example, include: multifilament stainless steel yarns; metallized aramid fibers; optical fibers for transmitting electrical data by acting as light waveguides; and glass or silica fibers for dielectric high frequency applications. Such highly functional yarns have been fabricated into fabrics, garments and apparel articles.

It is generally considered to be impractical to base a textile yarn solely on such high modulus filaments or on a combination yarn where the high modulus filaments are required to be a flex member of the yarn. Such high modulus filaments can typically be expected to exhibit low bending capability and poor flexibility.

Sources of stainless steel continuous multifilament fibers typically used in textiles include, but are not limited to: NV Bekaert SA, Kortrijk, Belgium; and Sprint Metal Groupe Arcelor, France. Depending on the number of filaments and the number of twisted yarns involved, these yarns usually have a filament diameter from about 6  $\mu\text{m}$  to about 12  $\mu\text{m}$ , and an electrical resistivity in the range of about 2 Ohm/m to about 70 Ohm/m. In general, these metal fibers exhibit a high force to break, typically in the range of about 20 N to about 500 N and relatively little elongation, typically less than about 5%. However, these fibers exhibit substantially no elasticity. In contrast, many elastic synthetic polymer based textile yarns stretch to at least about 125% of their unstressed specimen length and recover more than about 50% of this elongation upon relaxation of the stress.

Sources of plastic optical fibers for use in textiles include, but are not limited to: Toray Industries, Inc.; Mitsubishi Corporation; and Asahi Chemical. Typically, these fibers have diameters of about 0.5 to about 2 mm. Due to their construction, such fibers have the ability to transmit light along their length via total internal reflection, which light can then be converted into electrical energy or signals. This property of optical fibers tends to make them advantageous as compared to metal wires or coaxial transmission for data signal transmission, especially due to their relatively higher bandwidth, lower attenuation, lower noise, and lower cost.

Sources of metallized fibers include metallic coatings added on the surface of aramid fibers, such as Aracon® manufactured and sold by E.I. DuPont de Nemours. These yarns are based on stranded Kevlar® fibers, having an equivalent diameter to metal wire of about 54 AWG and electrical resistivity in the range of about 2 Ohms/m to about 9 Ohms/m. In general, these metallic fibers have a load to break of about 27 N to about 70 N and an elongation to break of less than about 5%.

## 2

Sources of inorganic quartz or silica fibers for use in textiles include, but are not limited to those made by Saint-Gobain (France). These fibers generally have filament diameters of about 1  $\mu\text{m}$  to about 25  $\mu\text{m}$ , a dielectric constant in the range of about 3 to about 7 in the frequency range up to about 10 GHz, and a loss tangent of about 0.0001 to about 0.0068 in the frequency range up to about 10 GHz. In general, these fibers exhibit a high tensile strength in the range of about 2000 N/mm<sup>2</sup> to about 6000 N/mm<sup>2</sup>, high tensile modulus of about 10 50,000 N/mm<sup>2</sup> to about 90,000 N/mm<sup>2</sup>, and relatively little elongation of about 2 to about 8%.

State of the Art: Plastic Optical Fibers in Textiles

Woven fabrics made by incorporation of optical fibers are known in the art. Typically, such optical fibers have an internal core and an external sheath. The external sheath has a lower refractive index compared to the internal core, which causes total internal reflection of light so that light travels solely through the internal core of the fiber. Light may be caused to escape from the surface of the fiber, thus creating an illuminating effect. There are two major directions disclosed for such effect: (1) attack of the fiber surface (mechanical or chemical), (2) deformation or bending of the fiber, at discrete locations along the fiber length.

15 (1) State-of-the-art Illumination by Optical Fibers Via Mechanical Attack

U.S. Pat. No. 4,234,907 to Maurice, discloses a light-emitting fabric woven with optical fibers for use in clothing, interior, or technical textiles. Optical fibers are woven in the warp direction crossed with normal textile fibers as weft threads. The optical fibers are illuminated at one end by a light source. Illumination from the surface of the fiber is achieved by making notches at the cladding till the inner core, the spacing of which becomes narrower as the distance from the light source increases so that there is a uniform distribution of light across the fabric. Analysis of such fabric makes it unsuitable for industrial manufacturing, as the notches weaken the fiber, making textile processing impossible, while the bundling of all fiber ends into a light source would require extreme fiber length extending out of the fabric.

20 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705

into a fabric. They were lighted through LEDs that could be used to light groups of fibers, each group representing one pixel of the matrix. By controlling the matrix through wireless telecommunication services, various patterns can be generated in the cloth, hence providing for an intelligent display. Although fine fiber diameters were used (about 0.5 mm), it was not optimal to create an X-Y network by introducing the fibers both in the weft and warp directions, as the fabric would be very rigid and the grid not very dense. Therefore, such fabrics would not be appropriate for typical clothing applications, where flexibility and freedom of movement of the fabric are of paramount importance. Further, special processing of the fibers is needed to transmit light from the surface of the optical fiber.

WO 2004/057079A1 to Laustsen, discloses a woven fabric with optical fibers that goes beyond the disclosure of U.S. Pat. No. 4,234,907 by allowing optical fibers to extend in mutually crossing directions in the fabric. According to the Laustsen reference, the fabric is hot rolled to compress and flatten the light guides, and further is laser treated to create partial ruptures at the surface of the optical fibers.

(2) State-of-the-art Illumination by Optical Fibers Via Bending

U.S. Pat. Nos. 4,885,663, 4,907,132, 5,042,900, and 5,568,964 to Parker et al., disclose fiber optic light emitting panel assemblies made of woven optical fibers. Light is caused to be transmitted from the optical fiber surfaces by deforming or bending the optical fibers at discrete locations along their length such that the angle of bend exceeds the angle of internal reflection. The optical fibers are typically woven in the warp direction, while fill threads are woven in the weft direction, although the fill threads are also allowed to be optical fibers. The output pattern of light is achieved by controlling the weave spacing and pattern of the optical fibers and fill threads. A portion of the light emitting area is sealed by adhering the optical fibers and fill threads together to hold the fill threads in position and keep the optical fibers from separating from the light emitting portion.

UK 2,361,431A to Whitehurst, discloses a fiber optic fabric for phototherapy, wherein light emitted from the surface of the optical fibers (including plastic and glass optical fibers) is directed towards a patient for the treatment of large area skin conditions for therapy, or cosmetic treatment. The inventor found that by weaving the optical fiber together with other fill yarns, the optical fiber bending around the fill fibers causes light to be refracted out of the optical fiber and hence out of the fabric. It is disclosed that when a large number of optical fibers is woven in this way, the fabric will emit light in a generally uniform distribution across the fabric. For the use of the fabric for phototherapy, it is very important that the fabric has flexibility to provide the necessary movement and comfort for the user, and that it follows the skin area that needs to be protected. However, it is known that fabrics based on optical fibers are rigid and tough for wearable clothing and will generally not allow movement of the fabric in the direction of optical fibers. Therefore, such a fabric may not provide for the desired flexibility or be optimum for the intended application.

(3) State-of-the-art Optical Fibers for Signal Transmission

U.S. Pat. No. 6,381,482B1 to Jayaraman et al., discloses a tubular knitted or woven fabric, or a woven or knitted 2-dimensional fabric, including integrated flexible information infrastructure for collecting, processing, transmitting, and receiving information concerning a wearer of the fabric. The fabric consists of a base fabric providing for wear comfort and an information component, which includes sheathed plastic optical fiber to provide a penetration detection means as well

as data transferring information. The fabric, consisting of the optical fibers, is then integrated into a garment structure by joining techniques such as sewing, gluing or attachment.

Optical fibers as sensors have also been used in textile composites to distribute sensing locally (point) or multiplexed (multi-point) exploiting intensiometric, interferometric, or Bragg grating principles. See X. M. Tao, *J. Text. Inst.* 2000, Vol 91 Part 1, No. 3, pp 448-459; and W. C. Du et al., *J. Compos. Struct.* Vol 42, pp. 217-230, (1998). Optical fibers can provide an effective means to determine quantitatively the distribution of physical parameters (e.g., temperature, stress-strain, pressure), and therefore may find uses in smart structures applications, such as monitors of manufacturing processes and internal-health conditions. In these developments, the embedded optical fibers also act as signal-transmission elements.

Stretch and recovery is considered to be an especially desirable property of a yarn, fabric or garment, which is also able to conduct electrical current, transmit data processing information, illuminate, sense, and/or provide electric field shielding. The stretch and recovery property, or "elasticity", is the ability of a yarn or fabric to elongate in the direction of a biasing force (in the direction of an applied elongating stress) and return substantially to its original length and shape, substantially without permanent deformation when the applied elongating stress is relaxed. In the textile arts, it is common to express the applied stress on a textile specimen (e.g., a yarn or filament) in terms of a force per unit of cross section area of the specimen or force per unit linear density of the unstretched specimen. The resulting strain (elongation) of the specimen is expressed in terms of a fraction or percentage of the original specimen length. A graphical representation of stress versus strain is the stress-strain curve, which is well-known in the textile arts.

The degree to which a fiber, yarn, or fabric returns to the original specimen length prior to being deformed by an applied stress is called "elastic recovery". In stretch and recovery testing of textile materials, it is also important to note the elastic limit of the test specimen. The elastic limit is the stress load above which the specimen shows permanent deformation. The available elongation range of an elastic filament is that range of extension throughout which there is no permanent deformation. The elastic limit of a yarn is reached when the original test specimen length is exceeded after the deformation inducing stress is removed. Typically, individual filaments and multifilament yarns elongate (strain) in the direction of the applied stress. This elongation is measured at a specified load or stress. In addition, it is useful to note the elongation at break of the filament or yarn specimen. This breaking elongation is that fraction of the original specimen length to which the specimen is strained by an applied stress which ruptures the last component of the specimen filament or multifilament yarn. Generally, the drafted length is given in terms of a draft ratio equal to the number of times a yarn is stretched from its relaxed unit length.

Elastic fabrics having conductive wiring affixed to the fabric for use in garments intended for monitoring of physiological functions in the body are disclosed in U.S. Pat. No. 6,341,504 to Istook. This patent discloses an elongated band of elastic material stretchable in the longitudinal direction and having at least one conductive wire incorporated into or onto the elastic fabric band. The conductive wiring in the elastic fabric band is formed in a prescribed curved configuration, e.g., a sinusoidal configuration. This elastic conductive band is able to stretch and alter the curvature of the conduction wire. As a result, the electrical inductance of the wire is changed. This property change is used to determine changes

in physiological functions of the wearer of a garment including such a conductive elastic band. The elastic band is formed in part using an elastic material, preferably spandex. Filaments of the spandex material, sold by INVISTA® North America Sà r. I., Wilmington, Del., under the trademark LYCRA®, are disclosed as being a desirable elastic material. Conventional textile means to form the conductive elastic band are disclosed, including: warp knitting, weft knitting, weaving, braiding, and non-woven construction. Other textile filaments, in addition to metallic filaments and spandex filaments, are included in the conductive elastic band. These other filaments include nylon and polyester.

While elastic conductive fabrics with stretch and recovery properties dominated by a spandex component of the composite fabric band have been disclosed, these conductive fabric bands are intended to be discrete elements of a fabric construction or garment used for prescribed physiological function monitoring. Although such elastic conductive bands may have advanced the art in physiological function monitoring, they have not been shown to be satisfactory for use in a way other than as discrete elements of a garment or fabric construction.

In view of the foregoing, it is believed desirable to provide high modulus functional textile yarns, including but not limited to conductive, fiber optic, and glass fibers, wherein such textile yarns have elastic recovery properties that can be processed using traditional textile means to produce knitted, woven, or nonwoven fabrics ("elastic functional yarns"). Further, it is believed that there is yet a need for fabrics and garments that are substantially constructed from such elastic functional yarns. Fabrics and garments substantially constructed from elastic functional yarns can provide stretch and recovery characteristics to the entire construction, conforming to any shape, any shaped body, or requirement for elasticity. It is further believed desirable to provide controlled loops (bends) of such high modulus functional fibers, either individually or within the fabric construction, so as to provide for special illumination effects, as in the case of optical fibers, or special electrical signals, as in the case of conductive fiber loops for inductive signal generation and transmission.

#### SUMMARY OF THE INVENTION

The present invention is directed to an elastic composite yarn comprising (a) a composite core member and (b) a composite covering member, wherein the composite core member comprises: (i) an elastic core member having relaxed unit length  $L$  and a drafted length of  $(N \times L)$ , wherein  $N$  is in the range of about 1.0 to about 8.0; and (ii) an inelastic functional core member having a fixed length of  $(N \times L)$ . The composite covering member comprises (i) at least one elastic covering member. Preferably, the composite covering member further comprises (ii) at least one inelastic covering member surrounding the elastic covering member. The composite covering member has a relaxed length that is greater than the drafted length  $(N \times L)$  of the elastic core member, such that substantially all of an elongating stress imposed on the composite yarn is carried by the elastic core member and the elastic covering member.

The present invention is also directed to methods for forming an elastic composite yarn. One method includes the step of first providing (a) a composite core and (b) a composite covering, wherein the composite core comprises: (i) a first elastic member having relaxed unit length  $L$  and a drafted length of  $(N \times L)$ , wherein  $N$  is in the range of about 1.0 to about 8.0; and (ii) an inelastic functional member having a fixed length of  $N \times L$ ; and the, composite covering comprises

(i) a second elastic member and (ii) at least one inelastic member. Further steps of the method include: drafting the first elastic member to a drafted length of  $(N \times L)$ , placing the inelastic functional member substantially parallel to and in contact with the drafted length of the first elastic member, and, thereafter, covering, twisting or wrapping in turns the composite covering about the drafted first elastic member and the inelastic functional member. The composite covering may be wrapped in the relaxed state or under tension. In addition, the at least one inelastic member of the composite covering may be wrapped in turns about the second elastic member, or the at least one inelastic member of the composite covering and the second elastic member may be twisted together.

It also lies within the scope of the present invention to provide a knit, woven or nonwoven fabric substantially constructed from functional elastic composite yarns of the present invention. Such fabrics may be used to form a wearable garment or other fabric articles substantially.

It further lies within the scope of the present invention to provide a novel means of forming loops (or bends) of the functional fiber member at discrete locations along the length of the fiber when such fiber is integrated into a knit, woven or nonwoven fabric. Such embodiments can further include a means of dynamically controlling such loops (for example, their size, bending angle, position) via the stretch and recovery function of such fabric.

#### BRIEF DESCRIPTION OF THE DRAWINGS

The invention will be more fully understood from the following detailed description, taken in connection with the accompanying drawings, which form a part of this application and in which:

FIGS. 1A and 1B show scanning electron micrographs (SEMs) of 100% stainless steel in parallel to Lycra® yarn type T-162C, single covered with a 22/7 dtex/7 filament flat nylon yarn twisted to the "S" direction at 500 turns per meter (tpm) in the relaxed state and in the relaxed state after break respectively;

FIG. 2 shows scanning electron micrographs (SEMs) of 100% stainless steel in parallel to Lycra® yarn type T-162C, double covered with a 22/7 dtex/7 filament flat nylon yarn twisted to the "S" and "Z" directions at 300 tpm and 200 tpm;

FIGS. 3A and 3B show scanning electron micrographs (SEMs) of 100% stainless steel in parallel to Lycra® yarn type T-162C, double covered with a nylon 44 dtex/20 filament textured yarn twisted to both the "S" and "Z" directions at 500 tpm in the relaxed state;

FIG. 4 shows a scanning electron micrograph (SEM) of 100% stainless steel in parallel to Lycra® yarn type T-162C, single covered with an elastified Lycra® yarn type T-902C (200 dtex, draft 5.2×) twisted to the "S" direction at 400 tpm;

FIGS. 5A and 5B show scanning electron micrographs (SEMs) of a Raytela® plastic optical fiber in parallel to Lycra® yarn type T-162C, single covered with a 22 dtex/7 filament flat nylon yarn twisted to the "S" direction at 333 tpm in the stretched and relaxed state, respectively;

FIGS. 6A and 6B show scanning electron micrographs (SEMs) of Raytela® plastic optical fiber in parallel to Lycra® yarn type T-162C, single covered with a 44 dtex/20 filament nylon yarn twisted to the "S" direction at 100 tpm in the relaxed state;

FIG. 7 shows a scanning electron micrograph (SEM) of a Raytela® plastic optical fiber in parallel to Lycra® yarn type T-162C, single covered with an elastified Lycra® yarn type T-902C (200 dtex, draft 5.2×) twisted to the "S" direction at 400 tpm;

FIG. 8 shows stress-strain mechanical property data indicating modulus definition for various high modulus functional fibers and traditional textile fibers.

FIG. 9 shows a scanning electron micrographs (SEM) in the relaxed state of a woven fabric produced in a Jaquard weaving loom type T.I.S. TMF 100, in which an elastic fiber optic yarn containing a Raytela® plastic optical fiber in parallel to Lycra® yarn type T-162C, single covered with an elastified Lycra® yarn type T-902C (200 dtex, draft 5.2x) twisted to the "S" direction at 400 tpm, was introduced in the weft direction and the warp directed was constructed by inelastic cotton yarns;

FIGS. 10A and 10B show scanning electron micrographs (SEMs) of the woven fabric shown in FIG. 9 that has been subjected to vaporization under a Hoffmann HR2A steam press table for about 1 minute in the relaxed and stretched state, respectively;

FIGS. 11A and 11B show scanning electron micrographs (SEMs) at different magnifications in the relaxed state of the woven fabric shown in FIGS. 10A and 10B that has been further subjected to heat setting through a Mathis laboratory heat stenter to about 180° C. for about 2 minutes; and

FIG. 12 is a schematic diagram of an elastic composite yarn according to the invention.

#### DETAILED DESCRIPTION OF THE INVENTION

In accordance with the present invention it has been found that it is possible to produce an elastic composite yarn containing high modulus or low bending fibers or yarns. Elastic composite yarns falling within the scope of the present invention comprise a composite core comprising: (a) an elastic core member (or "elastic core"); and (b) an inelastic functional core member, wherein the composite core is surrounded by at least one composite covering.

The elastic core member has a predetermined relaxed unit length (L) and a predetermined drafted length of (NxL), where N is a number, preferably in the range from about 1.0 to about 8.0, representing the draft applied to the elastic member. The inelastic functional core member has a fixed length of (NxL).

Elastic composite yarns falling within the scope of the present invention further include at least one composite covering. The composite covering includes: (i) at least one elastic covering member; and (ii) at least one inelastic covering member surrounding the elastic covering member. The composite covering has a relaxed length that is equal to or greater than the drafted length of the elastic core member, such that substantially all of an elongating stress imposed on the composite yarn is carried by the elastic core member and the elastic covering member.

#### The Elastic Core Member

The elastic core member may be implemented using one or a plurality (i.e., two or more) of filaments of an elastic yarn, such as that spandex material sold by INVISTA North America S.à.r.I. (Wilmington, Del., USA, 19880) under the trademark LYCRA®.

The drafted length (NxL) of the elastic core member is defined to be that length to which the elastic member may be stretched and return to within about five percent (5%) of its relaxed (stress free) unit length L. More generally, the draft (N) applied to the elastic core member is dependent upon the chemical and physical properties of the polymer comprising the elastic core member and the covering and textile process used. In the covering process for elastic members made from

spandex yarns a draft of typically is between about 1.0 and about 8.0, and most preferably about 1.2 to about 5.0

Alternatively, synthetic bicomponent multifilament textile yarns may also be used to form the elastic core member. The synthetic bicomponent filament component polymers are thermoplastic, more preferably the synthetic bicomponent filaments are melt spun, and most preferably the component polymers are selected from the group consisting of polyamides and polyesters.

A preferred class of polyamide bicomponent multifilament textile yarns are those nylon bicomponent yarns which are self-crimping, also called "self-texturing". These bicomponent yarns comprise a component of nylon 66 polymer or copolyamide having a first relative viscosity and a component of nylon 66 polymer or copolyamide having a second relative viscosity, wherein both components of polymer or copolyamide are in a side-by-side relationship as viewed in the cross section of the individual filament. Self-crimping nylon yarn such as the yarn sold by INVISTA North America S.à.r.I. under the trademark TACTEL® T-800™ is an especially useful bicomponent elastic yarn.

The preferred polyester component polymers include polyethylene terephthalate (PET), polytrimethylene terephthalate (PTT) and polytetramethylene terephthalate. The more preferred polyester bicomponent filaments comprise a component of PET polymer and a component of PTT polymer. Both components of the filament can be in a side-by-side relationship as viewed in the cross section of the individual filament. An especially advantageous filament yarn meeting this description is that yarn sold by INVISTA North America S.à.r.I. under the trademark T-400™ Next Generation Fiber. The covering process for elastic members from these bicomponent yarns involves the use of less draft than with spandex.

Typically, the draft for both polyamide or polyester bicomponent multifilament textile yarns is between about 1.0 and about 5.0.

#### The Functional Core Member

The term "functional core member" refers to one or more fibers that has at least one functionality or exhibits at least one property that extends beyond mechanical properties commonly associated with textile fibers. Functionalities or properties associated with such members can, for example, include fiber optic data transmission, dielectric high frequency applications (i.e., those using glass and/or silica fibers), activity under electrical, optical or magnetic fields, ability to convert energy from one form of energy to another, and sensory, monitoring or actuation applications.

The functional core member may, for example, be selected from the family of low bending modulus fibers, including stainless steel fiber, stainless steel yarn, conductive metallized aramid fibers, Plastic Optical Fiber (POF), and silica or glass optical fibers. The inelastic functional core member may, for example, have a force to break of greater than 2N in an elongation limit of less than 20% or a yield point of greater than 2N in an elongation limit of less than 20%.

The functional core member can further include: piezoelectric fibers from polymers (e.g., polyamide 7, polyamide 11), or from ceramic fiber composites; electrostrictive polymers; electrostrictive elastomers, ferroelectric fibers; magnetostrictive polymers or fiber composites; photonics fibers and nanocomposite fibers; thermo responsive (e.g., shape memory wires of polymers or metal alloys); photoluminescent and electrochromic fibers; and light sensitive liquid crystal containing fibers

In its most basic form, the functional core member comprises one or a plurality (i.e., two or more) strand(s) of functional fibers.

In an alternative form, the functional core member comprises a synthetic polymer yarn having one or more functional fibers(s) thereon. Suitable synthetic polymer yarns are selected from among continuous filament nylon yarns (e.g., from synthetic nylon polymers commonly designated as N66, N6, N610, N612, N7, N9), continuous filament polyester yarns (e.g., from synthetic polyester polymers commonly designated as PET, 3GT, 4GT, 2GN, 3GN, 4GN), staple nylon yarns, or staple polyester yarns. Such composite functional yarns may be formed by conventional yarn spinning techniques to produce composite yarns, such as plied, spun or textured yarns.

#### Composite Covering

The composite covering of the present invention comprises an elastic covering member and an inelastic covering member around or surrounding the elastic covering member. The length of the composite covering should be greater than, or equal to, the drafted length (NxL) of the elastic core member.

The elastic covering member may be comprised of any of the materials that can be used to for the elastic core member,

The inelastic covering member may be selected from non-conducting inelastic synthetic polymer fiber(s) or from natural textile fibers like cotton, wool, silk and linen. These synthetic polymer fibers may be continuous filament or staple yarns selected from multifilament flat yarns, partially oriented yarns, textured yarns, bicomponent yarns selected from nylon, polyester or filament yarn blends.

Optionally, the inelastic covering member may be a functional yarn with a tensile strength or less than 4N or a yield point of less 4N. Such functional yarns can include yarns with electrical or optical properties, such as a metal wire.

The inelastic covering member is preferably nylon. Nylon yarns comprised of synthetic polyamide component polymers such as nylon 6, nylon 66, nylon 46, nylon 7, nylon 9, nylon 10, nylon 11, nylon 610, nylon 612, nylon 12 and mixtures and copolyamides thereof are preferred. In the case of copolyamides, especially preferred are those including nylon 66 with up to 40 mole percent of a polyadipamide wherein the aliphatic diamine component is selected from the group of diamines available from INVISTA North America S.à r.l., (Wilmington, Del., USA, 19880) under the respective trademarks DYTEK A® and DYTEK EP®.

Making the inelastic covering member from nylon renders the composite yarn dyeable using conventional dyes and processes for coloration of textile nylon yarns and traditional nylon covered spandex yarns.

If the inelastic covering member is polyester, the preferred polyester is either polyethylene terephthalate (2GT, a.k.a. PET), polytrimethylene terephthalate (3GT, a.k.a. PTT) or polytetrahydroethylene terephthalate (4GT). Making the inelastic covering member from polyester multifilament yarns also permits ease of dyeing and handling in traditional textile processes.

The relative amounts of the functional core member and the composite covering are selected according to ability of the elastic core member to extend and return substantially to its unstretched length (that is, undeformed by the extension) and according to the functional properties of the functional core member. As used herein "undeformed" means that the elastic core member returns to within about +/- five percent (5%) of its relaxed (stress free) unit length L.

It has been found that any of the traditional textile process for single covering, double covering, air jet covering, entan-

gling, twisting or wrapping of elastic filaments and materials useful as functional filaments with materials useful in the composite covering is suitable for making the functional elastic composite yarn according to the invention.

In most cases, the order in which the composite core is surrounded by or covered by the composite covering is immaterial for obtaining an elastic composite yarn. A desirable characteristic of these functional elastic composite yarns of this construction is their stress-strain behavior. For example, under the stress of an elongating applied force, the composite covering, disposed about the composite core in multiple wraps (typically from one turn (a single wrap) to about 10,000 turns), is free to extend without strain due to the external stress.

If the composite yarn is stretched near to the break extension of the elastic core member, the composite covering is available to take a portion of the load and effectively preserve the elastic core member and the functional core member and prevent them from breaking. The term "portion of the load" is used herein to mean any amount from 1 to 90 percent of the load, and more preferably 10% to 80% of the load; and most preferably 25% to 50% of the load.

The composite core may optionally be sinuously wrapped by the composite covering. Sinuous wrapping is schematically represented in FIG. 12, where an elastic member 40, e.g., a LYCRA® yarn, is wrapped with an inelastic covering member 10, e.g., nylon, in such a way that the wraps are characterized by a sinuous period (P).

Specific embodiments and procedures of the present invention will now be described further, by way of example, as follows.

#### Test Methods

##### 35 Measurement of Fiber and Yarn Stress-Strain Properties

Fiber and Yarn Stress-Strain Properties were determined using a dynamometer at a constant rate of extension to the point of rupture. The dynamometer used was that manufactured by Instron Corp, 100 Royall Street, Canton, Mass., 02021 USA.

The specimens were conditioned to about 22° C. +/- about 1° C. and about 60% +/- about 5% R.H. The test was performed at a gauge length of about 5 cm and crosshead speed of about 50 cm/min. Threads measuring about 20 cm were removed from the bobbin and let relax on a velvet board for at least 16 hours in air-conditioned laboratory. A specimen of this yarn was placed in the jaws with a pre-tension weight corresponding to the yarn dtex so as not to give either tension or slack.

##### 50 Measurement of Fabric Stretch

Fabric stretch and recovery for a stretch woven fabric was determined using a universal electromechanical test and data acquisition system to perform a constant rate of extension tensile test. The system used was that from Instron Corp, 100 Royall Street, Canton, Mass., 02021 USA.

Two fabric properties were measured using this instrument: (1) fabric stretch and (2) fabric growth (deformation). The available fabric stretch was measured as the amount of elongation caused by a specific load between 0 and about 30 Newtons and expressed as a percentage change in length of the original fabric specimen as it was stretched at a rate of about 300 mm per minute. The fabric growth was measured as the unrecovered length of a fabric specimen which had been held at about 80% of available fabric stretch for about 30 minutes then allowed to relax for about 60 minutes. Where about 80% of available fabric stretch was greater than about 35% of the fabric elongation, this test was limited to about

11

35% elongation. The fabric growth was then expressed as a percentage of the original length.

The elongation or maximum stretch of stretch woven fabrics in the stretch direction was determined using a three-cycle test procedure. The maximum elongation measured was the ratio of the maximum extension of the test specimen to the initial sample length found in the third test cycle at load of about 30 Newtons. This third cycle value corresponds to hand elongation of the fabric specimen. This test was performed using the above-referenced universal electromechanical test and data acquisition system specifically equipped for this three-cycle test.

## EXAMPLES

Reference numerals present in the discussion of the Examples refer to the reference characters used in the accompanying drawing(s).

### Comparative Example 1

A 156 decitex (dtex) Lycra® yarn type T-162C was drafted by 3.8× its relaxed length, and fed in parallel to a 100% stainless steel yarn through a yarn covering I.C.B.T. machine model G307. The 100% stainless steel yarn was an endless multifilament yarn grade 316L consisting of two twisted threads with 275 filaments per thread and with a filament size of 12 obtained from Sprint Metal (France). This core composite yarn (consisting of Lycra® and stainless steel yarn) was single covered with a 22 dtex/7 filament flat nylon yarn twisted to the “S” direction at 500 tpm (turns per meter of drafted Lycra®). This yarn structure 10 is shown in FIG. 1A, with the Lycra® yarn 12 and stainless steel yarn 14 covered with the nylon yarn 16. As the yarn 10 is stretched, nylon cannot support the elastification and it breaks, as shown in FIG. 1B.

### Comparative Example 2

A core composite yarn of Lycra® and stainless steel yarn as in Comparative Example 1 was double covered with a 22 dtex/7 filament flat nylon yarn twisted to the “S” direction at 300 tpm (turns per meter of drafted Lycra®) and to the “Z” direction at 200 tpm. This yarn structure 20 is shown in FIG. 2, with the Lycra® yarn 12 and stainless steel yarn 14 covered by the nylon 16. Despite the fact that the yarn 20 was covered to a higher degree compared to Comparative Example 1 of the invention, as the yarn 20 is stretched, nylon cannot support the elastification and it breaks.

### Comparative Example 3

A covered yarn was produced as in Comparative Example 2, except it was twisted at 500 tpm in both the “S” and the “Z” directions. As the yarn is stretched, nylon cannot support the elastification and it breaks.

### Comparative Example 4

A covered yarn was produced as in Comparative Example 3, except that the nylon yarn used was a 44 dtex/20 filament textured yarn. The structure of this yarn 30 is shown in FIGS. 3A and 3B. Although a stronger nylon yarn 36 was used compared to Comparative Example 3, as the yarn 30 is stretched, nylon cannot support the elastification and it breaks.

12

### Example 1

A covered yarn was produced in a manner similar to that of Comparative Examples 1-4, except that the core composite yarn was single covered with an elastified yarn twisted to the “S” direction at 400 tpm. The elastified yarn was a double covered Lycra®& yarn (type T-902C, 200 dtex, draft 5.2×). The structure of this yarn 40 is shown in FIG. 4, with Lycra® yarn 42 and stainless steel yarn 44 covered by elastified yarn 46. As shown in FIG. 4, this yarn 40 presents a structure at the relaxed state comprising of straight segments, where the covered yarn holds the core composite yarn in the stretched state, and of loops of stainless steel. As the yarn 40 is stretched, the loops of stainless steel yarn tend to stretch parallel to the Lycra® core providing a totally stretched yarn that remains intact during stretching. This yarn can be further processed by standard textile processes.

### Comparative Example 5

A 156 decitex (dtex) Lycra® yarn type T-162C was drafted by 3.8× its relaxed length, and fed in parallel to a plastic optical fiber through a yarn covering I.C.B.T. machine model G307. The plastic optical fiber was type Raytela® from Toray of 610 dtex that comprised a fluorinated polymer clad and polymethyl methacrylate core. This core composite yarn was single covered with a 22 dtex/7 filament flat nylon yarn twisted to the “S” direction at 333 tpm (turns per meter of drafted Lycra®). This yarn structure 50 is shown in FIG. 5B, with Lycra® yarn 52 and plastic optical fiber 54 covered by nylon yarn 56. This structure 50 creates large loops of the optical fiber 54 up to a few cm in diameter during relaxing, as shown in FIG. 5B. As the yarn 50 is stretched, nylon cannot support the elastification and it breaks, as shown in FIG. 5A.

### Comparative Example 6

A covered yarn was made according to Comparative Example 5, except that it was single covered with a stronger nylon yarn (44 dtex/20 filaments) twisted to the “S” direction at 100 tpm. The structure of this yarn 60 is shown in FIGS. 6A and 6B, with Lycra® yarn 62 and plastic optical fiber 64 covered by nylon 66. The yarn 60 consists of straight parts as shown and loops of the optical fiber formed during relaxing the yarn. These loops can be as large as a few cm diameter so as to prohibit further processing of this yarn. As the yarn is stretched the nylon yarn breaks.

### Example 2

A covered yarn based on polymer optical fiber was formed as in Comparative Examples 5 and 6, except that the composite core yarn (consisting of Lycra® and optical fiber) was single covered with an elastified yarn twisted to the “S” direction at 400 tpm. The elastified yarn was a double covered Lycra® yarn (type T-902C, 200 dtex, draft 5.2×). The structure of this yarn 70 is shown in FIG. 7, with Lycra® yarn 72 and plastic optical fiber 74 covered by nylon 76. This yarn is composed of straight sections and small loops of optical fiber. As the yarn stretches, the loops of optical fiber straighten out with no break of the composite yarns, providing for a yarn that is processable by textile processes.

### Example 3

A woven fabric 90 was produced in a Jaquard weaving loom type T.I.S. TMF 100. Elastic Fiber Optic Yarn of

## 13

Example 2 was introduced in the weft direction of the fabric construction. The warp direction was constructed solely by inelastic cotton yarns 98. The fabric construction made was satin 16 to allow for maximum space between the fiber optic and the crossing warp yarns. The optical fibers introduced this way form loops of plastic optical fiber 94 that extend outside of the fabric, as shown in FIG. 9. In this case the fabric has limited stretch, for as the fabric is stretched the loops are slightly shortened but not to a complete extension.

## Example 4

The fabric of Example 3 was subjected to vaporization under a Hoffmann HR2A steam press table for about 1 min. The woven fabric was substantially shrunk, as caused by the influence of the elastic fiber optic yarns. In this state, the fabric 100 developed a substantial stretch and recovery function. In the relaxed state, this resulted in an increased size of the fiber optic 94 loops compared to the features observed in Example 3, as shown in FIG. 10A. In the stretch state, the loops were totally flattened out resulting in a total flat surface, as shown in FIG. 10B. Thus, by controlling the stretch and recovery of the fabric, there is a control of the magnitude of the fiber optic loop bending within the textile structure.

## Example 5

The fabric of Example 4 was subjected to heat setting through a Mathis laboratory heat stenter to about 180° C. for about 2 min. It was observed that the fabric 110 became totally rigid, and the fiber optic 94 loops totally flattened out as to create a flat fabric surface FIGS. 11A and B. It is thus possible, by controlling the heating of selecting parts of the fabric, to enforce straightening of the fiber optic loops, and therefore control of the fabric areas that can include loops or straight elements of fiber optic. This can introduce an additional degree of freedom compared to control induced by the weaving construction.

The examples are for the purpose of illustration only. Many other embodiments failing within the scope of the accompanying claims will be apparent to the skilled person.

What is claimed is:

1. An elastic composite yarn comprising:  
a composite core and a composite covering;  
wherein the composite core comprises:

(a) an elastic core member having relaxed unit length L and a drafted length of (N×L), wherein N is in the range of about 1.0 to about 8.0; and

(b) an inelastic functional core member having a fixed length of (N×L); and

wherein the composite covering comprises:

(a) at least an elastic covering member; and  
(b) at least one inelastic covering member surrounding the elastic covering member;

wherein the composite covering has a relaxed length that is greater than the drafted length (N×L), of the elastic core member, such that substantially all of an elongating stress imposed on the composite yarn is carried by the elastic core member and the elastic covering member.

2. The elastic composite yarn of claim 1, wherein the inelastic functional core member is selected from the group consisting of: stainless steel fibers, stainless steel yarns, plastic optical fibers, silica fibers, glass fibers, and metallized aramid fibers.

3. The elastic composite yarn of claim 1, wherein the inelastic functional core member comprises a functional yarn having at least one property selected from electrical, optical, and magnetic properties.

4. The elastic composite yarn of claim 1, wherein the inelastic functional core member has a modulus defined by

## 14

(a) a force to break of greater than 2N in an elongation limit of less than 20% or (b) a yield point of greater than 2N in an elongation limit of less than 20%.

5. The elastic composite yarn of claim 1, wherein the inelastic covering member comprises a textile fiber selected from the group consisting of: nylon, polyester, cotton, and wool.

6. The elastic composite yarn of claim 1, wherein the inelastic covering member comprises a functional yarn having electrical, optical or magnetic properties with a force to break or yield point of less than 4 N.

7. The elastic composite yarn of claim 6, wherein the inelastic covering member comprises a metal wire.

8. A method for forming an elastic composite yarn comprising:

(1) providing a composite core and a composite covering;  
wherein the composite core comprises:

(a) a first elastic member having relaxed unit length L and a drafted length of (N×L), wherein N is in the range of about 1.0 to about 8.0; and

(b) an inelastic functional member having a fixed length of N×L;

and wherein the composite covering comprises:

(a) a second elastic member;

(b) and at least one inelastic member;

(2) drafting the first elastic member to a drafted length of (N×L);

(3) placing the inelastic functional member substantially parallel to and in contact with the drafted length of the first elastic member; and

(4) wrapping, twisting, air jet covering, or core spinning in turns the composite covering about the drafted first elastic member and the inelastic functional member.

9. The method of claim 8, wherein the composite covering is wrapped about the first elastic member and the inelastic functional member in a relaxed state.

10. The method of claim 8, wherein the composite covering is wrapped about the first elastic member and the inelastic functional member under tension.

11. The method of claim 8, wherein the inelastic member of the composite covering is wrapped in turns about the second elastic member.

12. The method of claim 8, wherein the inelastic member of the composite covering and the second elastic member are twisted together.

13. The method of claim 8, wherein the second elastic member is air jet covered by the inelastic member of the composite covering.

14. The method of claim 8, wherein the second elastic member is core spun with the inelastic member of the composite covering.

15. A knitted or woven fabric comprising the elastic composite yarn of claim 1.

16. A method for controlling bending of electrical or optical fibers that are inelastic functional core member(s) in a composite yarn in a fabric, comprising:

(1) providing the fabric that includes one or more elastic composite yarns, said elastic composite yarns comprising

a composite core and a composite covering;  
wherein the composite core comprises:

(a) an elastic core member having relaxed unit length L and a drafted length of (N×L), wherein N is in the range of about 1.0 to about 8.0; and

(b) an inelastic functional core member having a fixed length of (N×L); and

wherein the composite covering comprises:

(a) at least an elastic covering member; and

(b) at least one inelastic covering member surrounding the elastic covering member;

**15**

wherein the composite covering has a relaxed length that is greater than the drafted length ( $N \times L$ ), of the elastic core member, such that substantially all of an elongating stress imposed on the composite yarn is carried by the elastic core member and the elastic covering member; and

(2) dynamically controlling bending or looping of the inelastic functional core member by stretching and relaxing the elastic composite yarn(s) in the fabric. 10

**17.** The method of claim **16**, further comprising differentiated heat setting the fabric.

**18.** A method for controlling bending of electrical or optical fibers that are inelastic functional core member(s) in a composite yarn in a fabric, comprising: 15

(1) providing the fabric that includes one or more elastic composite yarns, said elastic composite yarns comprising

a composite core and a composite covering;

**16**

wherein the composite core comprises:

- (a) an elastic core member having relaxed unit length  $L$  and a drafted length of  $(N \times L)$ , wherein  $N$  is in the range of about 1.0 to about 8.0; and
- (b) an inelastic functional core member having a fixed length of  $(N \times L)$ ; and

wherein the composite covering comprises:

- (a) at least an elastic covering member; and
- (b) at least one inelastic covering member surrounding the elastic covering member;

wherein the composite covering has a relaxed length that is greater than the drafted length ( $N \times L$ ), of the elastic core member, such that substantially all of an elongating stress imposed on the composite yarn is carried by the elastic core member and the elastic covering member; and

(2) heat setting at least a portion of the fabric to straighten at least some portions of the inelastic functional core member(s) in the fabric.

\* \* \* \* \*

UNITED STATES PATENT AND TRADEMARK OFFICE  
**CERTIFICATE OF CORRECTION**

PATENT NO. : 7,765,835 B2  
APPLICATION NO. : 11/719116  
DATED : August 3, 2010  
INVENTOR(S) : Eleni Karayianni et al.

Page 1 of 1

It is certified that error appears in the above-identified patent and that said Letters Patent is hereby corrected as shown below:

Title page, item [75], the address of inventor Philippe Chaudron should read  
-- Saint Julien en Genevois (FR); --.

Signed and Sealed this

Seventh Day of September, 2010



David J. Kappos  
Director of the United States Patent and Trademark Office